

April 20, 1943.

K. SCHWARTZWALDER ET AL

2,317,305

INSULATOR SEAL

Filed July 5, 1941



Fig. 1



Fig. 2

Inventor  
Karl Schwartzwalder &  
Robert M. Smith.  
By

Blackmar, Leonard & Clark  
Attorneys

## UNITED STATES PATENT OFFICE

2,317,305

## INSULATOR SEAL

Karl Schwartzwalder and Robert W. Smith,  
Flint, Mich., assignors to General Motors Corporation, Detroit, Mich., a corporation of Delaware

Application July 5, 1941, Serial No. 401,222

4 Claims. (Cl. 123—169)

Our invention has to do with providing a pressure tight seal between a ceramic body and metal. More particularly, it has to do with sealing electrodes in spark plug insulators.

In the spark plug industry today, it is proposed to make plugs in which a glass seal between the insulator and center wire or electrode provides a pressure tight connection by virtue of a bond which the glass forms with both the electrode and the insulator. For best results, it has been found that the metal of the electrode should have a low coefficient of expansion, and that the coefficient of expansion of the glass should be as close as possible to that of the metal. Low coefficient of expansion metals, with which a glass seal may readily be made to bond, are usually quite expensive. In our invention we have made it possible to retain the advantages of a metal which bonds readily with a glass seal and a less expensive metal having satisfactory properties as an electrode. We do this by making the center wire or electrode in two or more pieces, in which the metal which readily bonds with glass is joined to the metal electrode. Only so much of the former is used as may be necessary to insure a fluid tight seal.

It is an object of our invention to provide a seal between metal and a ceramic body which is strong, gas tight and permanent. This seal is made by the use of glass as the sealing element.

More specifically, it is the principal object of our invention to effect a seal between a spark plug insulator and its electrode by the use of glass in such a manner that the glass reacts with and bonds to both the metal and the ceramic body or insulator. This object is achieved without impairment of the operating efficiency of the plug.

Figure 1 of the drawing shows an insulator with the electrode and sealing material in place in the insulator before heat and pressure have been applied to complete the seal.

Figure 2 shows the completely assembled spark plug.

Referring to the drawing in detail, 10 indicates a spark plug insulator made of any suitable ceramic material. Thus the insulator may be of the porcelain type long in common use or the more recently developed sintered oxide or modified sintered oxide type. The insulator is provided with a counterbore or pocket 12 which may be threaded if desired. A hole or longitudinal bore 13 in the lower part of the insulator receives the center wire or electrode 14. Electrode 14 may be provided with a head or flange 16 which rests against the shoulder formed

at the juncture of longitudinal bore 13 and counterbore 12. The upper portion or terminal 18 of the center wire may be a screw which has a slightly smaller diameter than the counterbore of the insulator. Screw 18 is provided with a bore or recess 20 to receive a conductor or pilot wire 22. Wire 22 should be of a material which has a low coefficient of thermal expansion such as molybdenum, tungsten, invar and the like.

5 Pilot 22 is joined to electrode 14, as by welding, at the top of head 16 of the electrode. Electrode 14 is preferably made of a suitable heat resisting alloy material, such as a nickel alloy. Terminal 18 may be any good electrical conductor; we have found steel to be a satisfactory material.

A cylindrical pellet 23 of the cementing or sealing material fits over pilot wire 22. Pellet 23 is preferably a hard glass, such as a borosilicate glass; a satisfactory glass which is commercially available is that known as Pyrex. This glass unites with both the insulator and the metal pilot wire during the sealing operation. A second pellet 24 is provided to secure terminal 18 in the insulator. Pellet 24 preferably consists

20 of glass having a greater plasticity than glass pellet 23. A lead borosilicate glass combined with graphite or a metal has been found satisfactory for pellet 24. This glass may have the composition 50%  $B_2O_3$ -20%  $PbO$ -30%  $SiO_2$ . We

25 may provide a filler of powdered copper or Ticonderoga graphite. If pellet 24 is made from a mixture of glass and graphite we have found a satisfactory proportion to be 70% glass, 30% graphite. If it is a mixture of metal and glass, 30 we have found 50% metal, 50% glass to be satisfactory. The glass is crushed to pass a 150 mesh screen, and is mixed thoroughly with the filler and a suitable binder such as hydrogenated cotton seed oil, commercially known as Dritex. This

35 mixture may be formed into cylindrical pellets under pressure. Glass seals of this type are described in Patent 2,106,578 to Karl Schwartzwalder et al., issued January 25, 1938, Patent 2,071,571 to Hector Rabezzana et al., issued 40 February 23, 1937, and patent application Serial No. 343,808 of Karl Schwartzwalder et al., filed July 3, 1940.

The assembly shown in Figure 1 is next heated to a temperature of 1650° F. or higher to make 45 the glass plastic. Pressure is then applied to screw 18 to force it into the desired position, shown in Figure 2. This pressure causes pellet 23 to flow and react with insulator 10 and pilot wire 22. The condition of pellet 23 after flowing under pressure is indicated at 23a in Figure 2.

Sealing material 24 is likewise caused to flow between screw 18 and the insulator, as shown at 24a of Figure 2. After the assembly has cooled, a compression or vacuum tight seal exists between electrode 14 and insulator 10, and the whole structure is held rigidly together so that no compression leakage occurs even after the most severe usage.

We claim:

1. A ceramic body having a passageway therethrough, a recessed terminal in said passageway, a conductor in the passageway and in contact with the terminal through its recesses, said conductor having a low coefficient of thermal expansion, a fluid-tight seal of hard glass bonded to the conductor and the ceramic body, and a glass seal of greater plasticity than the first glass seal between the insulator and the terminal.

2. A ceramic body with an opening therethrough, an enlargement in said opening defining a shoulder, an electrode in the opening having a relatively high coefficient of thermal expansion, a flange on the electrode abutting on the shoulder, a wire having a low coefficient of thermal expansion joined to the electrode, a recessed terminal in the enlargement having contact in its recess with the wire, a fluid-tight seal of hard glass bonded to the wire and the ceramic body, and a second seal between the terminal and

ceramic body, said second seal including glass having greater plasticity than the first glass seal.

3. In a spark plug, an insulator having an opening therethrough, a terminal in said opening, an elongated recess in said terminal, a wire in said opening and in contact with the terminal at the inner end of said recess, a fluid tight seal having a bonded connection to the wire and the insulator, and a second seal between the insulator and the terminal.

4. In a spark plug, a ceramic insulator having an opening therethrough, a terminal in said opening, an electrode in said opening having a relatively high coefficient of thermal expansion, a conductor having a low coefficient of thermal expansion joined at one of its ends to said electrode and having its other end in electrical conducting relationship with the terminal, a fluid-tight seal of hard glass bonded to the conductor and to the ceramic insulator, said hard glass having substantially the same coefficient of thermal expansion as said conductor, and a second seal between the insulator and the terminal, said second seal including glass having a greater plasticity than the hard glass seal.

KARL SCHWARTZWALDER.  
ROBERT W. SMITH.

CERTIFICATE OF CORRECTION.

Patent No. 2,317,305.

April 20, 1943.

KARL SCHWARTZWALDER, ET AL.

It is hereby certified that error appears in the printed specification of the above numbered patent requiring correction as follows: Page 2, first column, line 13, claim 1, for "recesses" read --recess--; and that the said Letters Patent should be read with this correction therein that the same may conform to the record of the case in the Patent Office.

Signed and sealed this 1st day of June, A. D. 1943.

Henry Van Arsdale,

(Seal) Acting Commissioner of Patents.